

## 1

3,072,541  
DEVELOPER

Benjamin L. Shely, Mahtomedi, and Bryce L. Clark, St. Paul, Minn., assignors to Minnesota Mining and Manufacturing Company, St. Paul, Minn., a corporation of Delaware

No Drawing. Filed Oct. 17, 1958, Ser. No. 767,788  
5 Claims. (Cl. 204—18)

This invention relates to the formation of permanent visible reproductions of light-images on photoconductive surfaces by methods involving electrolysis at the exposed light-sensitive surface. It has particular reference to improved electrolytic developer solutions employed in such method.

Methods have recently been devised for electrolytically forming visible reproductions of light-images on strongly photoconductive light-sensitive copy-sheet materials. Apparatus for carrying out such methods, particularly in making enlarged reproductions of microfilm copies of graphic originals, has also been made available. Typically, there is involved the brief irradiation of a sensitive copy-paper with a light-image corresponding to the copy desired, and the subsequent electrodeposition at the conductive light-struck areas of a metallic image-forming material as the copy-paper is withdrawn from the irradiation area. The copy is obtained in substantially dry form, since only a surface application of developer solution is applied. No subsequent treatment, such as heating, washing, or subjecting to the action of chemical vapors, is required. Completed reproductions of microfilm transparencies or other graphic originals may be produced at a rate of ten or more per minute.

A recommended form of light-sensitive copy-paper for use with the apparatus and method hereinabove identified consists of a strongly photoconductive zinc oxide surface coating on a metallized or metallic conductive backing or sheet material. Such a sheet, having an 0.8 mil coating of four parts by weight of zinc oxide and one part of polymeric insulating binder on a laminate of paper and aluminum foil, typically has a conductivity value, measured as hereinafter described, of at least about  $10^{-7}$  mho/cm. and preferably not less than about  $10^{-6}$  mho/cm. Under equilibrium dark conditions the conductivity value is not higher than about one-twentieth of the conductivity value under illumination, and ordinarily is much lower.

The conductivity value is measured as follows: A small sample of the sheet material is insulated at back and edge areas with a nonconductive waterproof covering, e.g., of plastic adhesive tape, an electrical connection to the conductive metallic substrate being provided. The sample is suspended in a transparent glass cell containing 200 ml. of a solution of tenth-molar ammonium sulfate and facing an open frame electrode serving as the anode. Current flow per unit area through the measured thickness of the coating under an applied voltage is measured both with the sample under equilibrium dark conditions and when illuminated. A potential of 10 volts is convenient but not critical. Values at several thicknesses of coatings may be determined and the value at a standard thickness of 0.8 mil obtained by interpolation. Illumination is provided from a 500 watt incandescent-filament lamp, i.e. at an intensity of about 1300 foot-candles. The photoconductivity value is calculated from the values thus obtained.

As electrolytic developer solutions for use in the above-identified apparatus and method, there have been suggested solutions of salts of platable metals, e.g. copper sulfate, nickel chloride, or cadmium nitrate solutions. An initially visible image may indeed be formed with each of these; but for one reason or another the result-

## 2

ing copy has not been entirely satisfactory. For example, with platable base metals the image is found to fade rapidly when the copy is exposed to high humidity. Since some moisture is unavoidably present at the surface of the sheet following image development, conditions are normally unfavorable for image permanency. Furthermore, although electrolysis of many such salts does initially produce a visible image, the quality of the image is low. The image areas obtained are in most cases grayish rather than the desired dense black, and the copy lacks contrast. The noble metals produced no better, or even less effective images. Silver nitrate, for example, produces a yellowish-brown image and a darkened background. Gold salts likewise produce images of low density. Solutions of gold and platinum salts are highly corrosive to metallic structural components and prohibitively expensive for most copying purposes.

Electrodeposition of metals from corresponding salt solutions, as in the electroplating art, is frequently improved in one respect or another by the inclusion of various additives in the plating solution. For example, soluble cyanides are normally added in small amounts to silver-plating baths to improve the brightness and permanence of the plate. It might therefore be expected that the substitution of typical metal-plating solutions for the simple salt solutions would likewise improve the quality of the image obtainable in the electrolytic reproduction process hereinabove identified. It has been found, however, that electroplating formulations in general offer inadequate improvement over the less complicated simple salt solutions in such process. Formulations employing base metals provide image areas of somewhat improved initial density and contrast, but the images are not permanent and fade or disappear rapidly when the sheet is held at high humidities. The cyanides are additionally highly undesirable because of their poisonous nature, since the residual unreacted salts, or residues resulting from the electrolytic decomposition of such salts, in all instances remain on the copy-paper rather than being removed, as in normal metal plating operations, by subsequent washing.

On the other hand, additives which are employed to provide increased brightness of the metallic plate might appear likely to be disadvantageous in the electrolytic development of light-images on a white base, where a dense black rather than a bright metallic deposit is normally desired.

It has now been found that certain normally stable soluble electrolyzable complexes of platable metals provide electrolytic developer solutions with which by methods noted hereinbefore, may be obtained dense dark-colored image-forming deposits of a high degree of permanence, all as demonstrated by the following illustrative but non-limitative specific examples.

| Example 1      |  | Parts by weight |
|----------------|--|-----------------|
| Silver nitrate |  | 1.00            |
| Thiourea       |  | 1.35            |
| Acetamide      |  | 4               |
| Water to make  |  | 100             |

The several components are mixed together at room temperature, forming a clear solution, which is placed in the metal reservoir of an electrolytic printing device. A thin strip of cellulosic sponge is partly submerged in the solution. A sheet of photoconductive zinc oxide coated copypaper as described hereinbefore is exposed to a light-image, and the exposed surface then drawn slowly across the strip of sponge while the conductive backing of the sheet and the metal reservoir are connected to the poles of a battery. The sheet is thereby made the cathode of an electrolytic cell. As the sensitized sheet contacts the

solution in the sponge, a dense black deposit is formed at the conductive light-struck areas. The print shows no visible decrease in contrast or image density after several weeks in a high humidity test chamber at normal room temperature.

Pressure between sheet and sponge, width of sponge face, and other factors are so controlled as to provide a minimum deposit of solution on the sheet consistent with the effective formation of the image. The amount applied is insufficient to appear as a liquid layer on the sheet as it is taken from the printer. The moisture is soon volatilized, the residual non-volatile material remaining on or in the oxide-coated surface.

When a dilute solution of silver nitrate is employed in the foregoing procedure as the electrolytic developer solution, the image areas are yellowish-brown in color and the background areas are noticeably darkened. The resulting reproduction is essentially stable, showing no observable change or prolonged storage at high humidity, but has low contrast and is not a desirable print.

When combined as described in Example 1, silver nitrate and thiourea form a normally stable, soluble, electrolyzable complex which can be separated from the solution in crystalline form by cooling to somewhat below 15° C. The washed and dried crystals are found to melt at about 156° C. and to be substantially free of acetamide. Dissolved in appropriate ionizable solvent, the pure crystalline complex likewise provides a stable liquid electrolytic developer solution useful in forming permanent dense dark-colored image-forming deposits on photoconductive copy-paper.

In the absence of thiourea, the acetamide shown in Example 1 is itself instrumental in increasing the density and improving the appearance of the image-forming deposits obtained with the silver nitrate developer solution. However the complexes formed with this compound are relatively less stable and presumably are not present in the solution of the example, although such complexes may be present when less than three mols of thiourea are employed. The acetamide is in any event helpful in forming the stable complex from silver nitrate and thiourea and, since it imparts no harmful effects, is ordinarily retained in the developer solution.

Maximum image density is obtained with the thiourea-silver nitrate system at the three-to-one molar ratio. Increasing the amount of thiourea, for example from 1.35 up to 4.0 parts in Example 1, does not impair either the density or the permanence of the image-forming deposits when properly formed, but has caused noticeable fading in cases where larger than usual amounts of the solution were applied and allowed to remain on the copy-paper.

The image-forming deposits obtained with the thiourea-silver nitrate complex have been observed to be composed primarily of metallic silver (or its oxide) and silver sulfide. The image areas therefore have much in common with images produced by silver halide photography; and the appearance of the finished prints furthers this comparison. For this reason, stable soluble electrolyzable complexes of silver salts and sulfur-containing complexing agents are ordinarily preferred. Complexes of other platable metals with these and other complexing agents, and which are stable in solution form and on electrolysis produce permanent dark-colored dense image-forming deposits, are also useful. Aqueous systems will ordinarily be found preferable, but other ionizing solvents are known with which effective solutions of many of these various complexes may be prepared. For example, glycerine and formamide may be used where the amount applied is so small in relation to the thickness and absorbency of the copy-paper as to avoid any necessity of subsequent solvent evaporation.

#### Example 2

A 2% solution of  $(HAuCl_4 \cdot 3H_2O)$  is applied in a

thin coating on a sheet of photoconductive zinc oxide coated copy-paper which has been exposed to a light-image. The solution is applied by wiping with a cellulosic sponge dampened with the solution and in conductive contact with a gold electrode through which contact is made to a suitable source of potential and to the conductive backing of the copy-paper. Plating occurs at the cathodic light-exposed areas, which are thereby rendered visible. When tested with a "Densichron" optical density measuring instrument, the proportion of the incident light normally reflected by the untreated copy-paper which is absorbed by the thus developed image areas is found to be 37%. Although the image is stable, remaining unchanged in density after one week at high humidity, the density is undesirably low for effective readability.

An aqueous solution prepared with 2% of gold chloride in conjunction with 4% of acetamide is similarly tested. The image areas have a density of 68% as first prepared, and 67% after one week at high (98%) humidity. Addition of 2% thiourea to the solution results in the formation of developed image areas having a density of 81% and likewise dropping only to 80% after one week at high humidity. In both instances excellent reproductions are obtained, and the image areas remain dark-colored and distinct in the presence of substantial residues of developer materials and at high humidities.

What is claimed is as follows:

1. The process for producing permanent, dense image-forming deposits on light-exposed areas of strongly photoconductive photosensitive copy-paper having a photoconductive coating on an electrically conductive backing, said copy-paper being capable of electrolytic image reproduction thereon, which comprises electrolyzing at the conductive light exposed areas of said photoconductive coating a stable liquid electrolytic developer solution consisting essentially of a stable solution in an ionizing solvent of a soluble electrolyzable complex of a silver salt and a thiourea in a 1:3 molar ratio, said electrically conductive backing being connected as cathode.

2. The process of claim 1 in which said ionizing solvent is water.

3. The process for producing permanent, dense image-forming deposits on light-exposed areas of strongly photoconductive photosensitive copy-paper having a photoconductive zinc oxide coating on an electrically conductive backing, said copy-paper being capable of electrolytic image reproduction thereon, which comprises electrolyzing at the conductive light exposed areas of said photoconductive coating a stable liquid electrolytic developer solution consisting essentially of a stable solution in an ionizing solvent of a soluble electrolyzable complex of a silver salt and a thiourea in a 1:3 molar ratio, said electrically conductive backing being connected as cathode.

4. The process of claim 3 in which said ionizing solvent is water.

5. The process of claim 3 in which said electrolytic developer solution also contains acetamide.

#### References Cited in the file of this patent

#### UNITED STATES PATENTS

|           |                      |                |
|-----------|----------------------|----------------|
| 1,857,507 | Hickman et al. ----- | May 10, 1932   |
| 1,902,213 | Brockway -----       | Mar. 21, 1933  |
| 1,903,860 | Gockel -----         | Apr. 8, 1933   |
| 2,083,249 | Thomson -----        | June 8, 1937   |
| 2,186,859 | Digby -----          | Jan. 9, 1940   |
| 2,443,119 | Rubin -----          | June 8, 1948   |
| 2,692,190 | Pritikin -----       | Oct. 19, 1954  |
| 2,854,386 | Lyman et al. -----   | Sept. 30, 1958 |

#### FOREIGN PATENTS

|         |                 |               |
|---------|-----------------|---------------|
| 151,971 | Germany -----   | Dec. 8, 1902  |
| 215,754 | Australia ----- | June 23, 1958 |

UNITED STATES PATENT OFFICE  
CERTIFICATE OF CORRECTION

Patent No. 3,072,541

January 8, 1963

Benjamin L. Shely et al.

It is hereby certified that error appears in the above numbered patent requiring correction and that the said Letters Patent should read as corrected below.

Column 1, line 20, for "if" read -- of --; column 2, lines 20 and 21, for "variout" read -- various --; line 26, for "improved" read -- improve --; column 2, Example 1, line 4 thereof, for "Wate" read -- Water --; column 3, line 19, for "or" read -- on --.

Signed and sealed this 2nd day of July 1963.

(SEAL)

Attest:

ERNEST W. SWIDER  
Attesting Officer

DAVID L. LADD  
Commissioner of Patents